

Jan. 20, 1931.

A. R. BAKER ET AL

1,789,615

PHOTOGRAPHIC LINE PRINT AND METHOD OF MAKING THE SAME

Filed July 8, 1929

Fig. 1.



Fig. 2.



Fig. 3.



Fig. 4.



Fig. 5.



INVENTORS.

Arthur R. Baker

Walter N. Baker

Thomas H. Ferguson

ATTORNEY.

Fig. 6.



## UNITED STATES PATENT OFFICE

ARTHUR R. BAKER AND WALTER N. BAKER, OF CHICAGO, ILLINOIS

## PHOTOGRAPHIC LINE PRINT AND METHOD OF MAKING THE SAME

Application filed July 8, 1929. Serial No. 376,744.

The present invention relates to photographic line printing of the class wherein the work, that is, the delineations, or lines and dots which go to make up the image, is placed upon a basic coating of collodion, lacquer, or like substance, and wherein said basic coating between the lines and dots is left exposed to atmosphere.

This class of printing is in contrast to that where the sensitive coating, after being photographically exposed, developed and fixed, is not removed, but is allowed to remain covering the basic coating.

Prints of the former class, as heretofore made, do not present a surface upon which additions to the image may be readily drawn or written. Since it is the basic coating of collodion, lacquer, or the like, which must receive the ink or lead, if additions are to be made, it is obvious that such coating must be able to receive and retain the applied material. But in prior art prints of the class mentioned this has not been the case; the basic coating will not satisfactorily receive and hold the added markings.

Another condition to be found in prior art prints of the class in question, is the brittleness of the structure of the work. By bending such prints back and forth a number of times at one point in the work, the latter may be badly mutilated. This mutilation is the result of the chipping off, or the breaking up, of the material of the work. Its rupture spoils the image.

The principal object of the present invention is to provide a new print of the class mentioned wherein desired additions may be readily made to the image, and wherein the lines and dots, or either of them, constituting the work, may not be easily removed or mutilated in the manner pointed out. The invention includes not only the prints having these characteristics, but the method of producing the same.

In carrying out our invention, we start with a print having the basic coating mentioned, and apply thereto a solvent of the basic coating material, and then remove the resulting solution or softened material, so as to bare the base between the lines and

dots, the solution, meanwhile, being spread over these lines and dots to strengthen and protect them. The bared, or substantially bared, base can then be written or drawn upon to enlarge or modify the image of the print, the base itself being sufficiently free of the basic coating and being itself of such material that it will readily and effectively take the ink or lead of the additions. The smearing of the dissolved basic material over the lines and dots, toughens and hardens them. The result is that the new print may be easily drawn, or written, upon for the purpose of making additions to its image, and rough handling of the print does not chip, break off, or otherwise mutilate the lines and the dots constituting the work originally on the print.

In our practice of the invention we have commonly applied the same to prints formed upon a transparent or translucent base, and then the resulting print, produced in accordance with the present invention, can itself be used for making additional prints.

An important part of the present invention, which may have a wide application in silver photography, resides in the fact that when the sensitive coating we have been describing is one containing a bichromate, with its holding qualities, and a silver salt, with its light sensitive qualities, the solvent for the basic coating, which we have also mentioned, suffices to fix the exposed delineations of the sensitive coating without the need of the usual photographic silver salt fixing solution, such as hypo, ferricyanide of potash, and the like. The use of our solvent thus frees the product from many objections which result from the use of these chemicals.

Having presented these general views of the nature and character of the invention we may now pass to a detailed disclosure of a preferred embodiment of the same. This is set forth in the following description and the accompanying drawing wherein the steps of the method and the character of the resulting product are presented. For the scope of the invention, reference should be had to the appended claims.

In said drawing, Fig. 1 is a plan view of a

base coated as heretofore described for the production of a print which will constitute the basis for the practice of our invention, portions of the coatings being removed to show their relative positions; Fig. 2 is a side elevation of the same, also showing portions of the coatings removed; Fig. 3 is a plan view showing the image developed and fixed, and ready for the steps of our new method; Fig. 4 is a vertical section of said developed and fixed print, the plane of section being indicated by the line 4—4 of Fig. 3; Fig. 5 shows the previous structure treated by the basic coating solvent and showing the resulting dissolved material removed from the base between the lines, and spread over the work as a protective coating to the same, all as contemplated by the present invention; and Fig. 6 is a similar view of the right-hand portion of the same structure illustrating the removal of material applied to, or impregnated in, the base as well as the removal of material of the basic coating. Throughout these views like characters refer to like parts.

28 The several views of the drawing are in measure diagrammatic. They also show the parts upon a greatly enlarged scale. All this is done with a view to clearness.

30 As previously pointed out the print structure which constitutes the basis for the application of our invention, consists of a base A, a first coating B, and a second coating C. The base A may be composed of a stiff or flexible material. However, in the practice of our invention we find it desirable to employ a flexible material, commonly a fabric impregnated with starch, such as tracing cloth. Obviously, the flexible material may be either paper or cloth. The use of a translucent base, 40 which we commonly use, enables the resulting print to be used as a positive for printing other prints, as before noted.

45 The second coating B is a water-proofing coating of lacquer, collodion, compounds of lacquer, compounds of collodion, or mixtures of these materials.

50 The third coating C is a light sensitive coating having a bichromate as a basic ingredient. Such bichromate may be a gum bichromate, a glue bichromate, a gelatin bichromate, or an albumen bichromate. Indeed, any of the bichromates commonly employed in bichromate photography would be suitable for this basic ingredient. The other elements of the coating C may vary greatly, but they divide themselves into two classes, viz: those that include silver salts on the one hand, and those that include pigments and dyes on the other. As illustrative of silver photography, these elements may be silver nitrate, silver chloride, potassium citrate, potassium bromide, potassium iodide, ammonium bichromate, potassium bichromate, and sodium bichromate, variously compounded. These mentioned 60 elements are merely illustrative, and persons

familiar with silver photography will appreciate the value of the different substances, and will be able to combine these and others in suitable ways to give proper photographic results. As illustrative of the class employing 70 pigments and dyes for bringing out the image, we may refer to the ingredients mentioned in our previous Patent 1,704,356, dated March 5, 1929. As there pointed out, pigments of different kinds for different colors 75 may be used. The same is also true of dyes. Different dyes may be employed for different colors. In the present case the coating C, whether employing the pigments, dyes, or silver salts, includes one or more of the bichromates, as stated.

80 The structure built up by the base A and the coatings B and C constitute a plate, film or the like, for the receiving of the photographic images. If the strip or sheet thus constituted is positioned back of a negative having the image of Fig. 3 upon it, and the plate is properly exposed to light, then portions of the upper coating C will be acted upon by the light and chemically changed. 85 Then as soon as the strip is properly treated the image will show forth, as in Fig. 3.

89 For the treatment of the pigment or dye coating, in accordance with the process of our aforesaid patent, it is only necessary to wash off the print with water. This washing will dissolve and carry away that portion of the coating C which has not been chemically changed by the light. When it comes to treating the coating C where the latter includes a silver salt it is necessary to use a developer, such as is commonly used in silver photography, to produce a change in the color of those portions of the coating which has been acted upon by the light. In the case of the silver compound, the image will remain just as in the case of the pigment or dye compound, but the silver salt requires the use of a developer which the pigment or dye does not. In both cases the washing of the print with water will carry away those portions of the coating which are not fixed to show the image. This is clearly illustrated in Fig. 4 where the fixed portions C<sup>1</sup> and C<sup>2</sup> of the image stand up above the surface of the basic coating B.

105 But, as we shall see later, when our solvent is used to remove the basic coating B, it is not necessary to use a fixing solution on the silver salts coating C. This is an incidental but novel feature in our silver photography development. This point should be borne in mind when preparing silver prints for the subsequent steps of our invention. It may be noted, however, that the use of hypo, 110 ferricyanide and the like for fixing purposes prior to using the steps of our invention is not objectionable. Our method can be carried out just as well, and with just as good results, no matter whether the fixer be used 115

or not. But obviously its use, being unnecessary, better be omitted if the prints are to be subjected to the application of our solvent.

As has been indicated, a print, such as shown in Figs. 3 and 4, produced by any of the methods just described, is the starting point for the practice of our invention. Starting with the print in this form, we may proceed with a description of our invention.

10 In practice it is found that the coating B will not take the ink of the pen or the lead of the lead pencil to any advantage. The surface of this coating is glassy and not of the right texture to draw or write upon. 15 Therefore, if it is desired to add to the image, to the portion C<sup>1</sup>, for example, it is difficult to do so because of the inability of the coating B to take and hold the substance applied or sought to be applied. Furthermore, if we 20 consider the print in this form, it is easy, as before stated, to bend the print back and forth and thus mutilate the material of the coating C which forms part of the image. This destroys the clearness of the image and 25 hence reduces the value of the print.

In order to meet these difficulties, we apply to the surface of the print a solvent of the coating B. This solvent is preferably a mixture of alcohol and ether; commonly, one part 30 by volume of alcohol is mixed with one part by volume of ether, although we have found in practice that these proportions may be varied through a wide range without objectionable results. We have also found that 35 where the print is of the pigment or dye class, more alcohol may be used than ether. On the other hand, where the print is of the silver class the proportions just mentioned are preferable. Other solvents may also be employed 40 if desired but the ones mentioned are quite satisfactory, being both effective and economical.

This solvent may be applied in different ways. A small piece of cotton batting 45 dipped in the solution may be rubbed lightly over the surface of the print a number of times and, preferably, in different directions. The effect is to soften up the material of the coating B and bring it 50 practically into solution, depending, of course, upon the amount and strength of the solvent applied. The moving of the piece of batting over the surface will also wipe up the coating B from the surface of the base A between the lines and dots, and clean the same 55 more or less perfectly at those points, while at the same time carrying the solution over the work already on the print. The effect is shown particularly in Fig. 5. There the 60 coating B is practically removed at all points except where it underlies, or substantially underlies, the work C<sup>1</sup> and C<sup>2</sup>. The surface of the base A is left bare, or practically so, wherever the coating B has been removed. 65 As the dissolved material is removed from

between the lines it is applied as a coating B<sup>1</sup> to the work C<sup>1</sup> and C<sup>2</sup>, as clearly illustrated.

Removing the basic coating B from between the lines has the effect of sharpening the edges of the lines and brightening the 70 print. Often stains and sediment are present in or lodged upon the coating B and the cleaning of the coating from the base removes all stains and sediment. The stains often come from photographic chemicals and the sediment is present in the form of visible particles embedded in the coating. The application of the solvent in the way described also takes away the shiny effect of the lines, often present, and it may be applied so as to 75 remove any sediment on the lines themselves. Likewise, where the lines are too wide because of overexposure, they may be brought to proper width by repeating the applications of the solvent to the lines, usually brushing 80 over them from the sides of the lines for this purpose as is done in photolithographing and other like work.

The application of the solvent to the coating B may be by wiping, as just described, 90 scraping, spraying, or otherwise, as desired. It is only necessary in each of these methods to remove the dissolved coating from between the lines and to apply the same to the lines 95 and dots.

Where the base A is coated or impregnated with a material which will be dissolved by the solvent of the coating B, as would be the case with tracing cloth, then some of the material of the coating, such as the starch of 100 the tracing cloth, would be more or less mixed with the material which forms the coating B<sup>1</sup>. In such event the removal of soluble material from the base A will more fully expose the fibre of the base. An attempt has been 105 made to illustrate this action in Fig. 6. There the dotted line 10 shows the original surface of the base and the full lines below it represent its surface after portions of 110 the starch or like filling have been dissolved out and wiped away. The impregnating material thus wiped away mingles with the removed portions of the coating B to form the work covering B<sup>1</sup>. Obviously, a base A 115 having no filling or impregnating material would not have its surface changed in this way and the coating B<sup>1</sup> would be that which resulted solely from the dissolution or softening of the material of the basic coating B. 120

The removal of the basic coating from between the lines also renders the finished print more pliable where it is made upon a flexible base A. This necessarily results from the removal of a large part of the basic coating B 125 which is relatively stiff when thoroughly dried. Its removal also leaves the coated base thinner. The resulting greater flexibility of the print prevents the peeling off of the basic coating, as has so often been the 130

case heretofore with prior art prints of this class.

As incidental to the practice of our invention as just described, is the important fact that where the coating C is made up of silver salts in accordance with well-known practices in silver photography, the use of our solvent, as heretofore described, does away with the need of using the fixing agents commonly employed in that branch of photography, such as hypo and ferricyanide of potash. The use of our solvent upon the silver salt coating C performs the necessary reducing and fixing functions and renders the print permanent without the use of the customary fixing agents. This results in making the photographically printed lines more permanent, as there will be no traces of the hypo or ferricyanide left in the lines to cause the print to deteriorate as is commonly the case where they are used, the prints being bleached by the light as they grow old and the background becoming yellowish in color. So in the case of the silver salts coating C, all that is necessary is to use the developer, water and our solvent; and in the case of the dye or pigment coating C, merely use water and our solvent. We do not say that our solvent is a substitute for hypo and ferricyanide in silver photography but it is such a substitute where the coating C is a silver salt compound on a coating of the character of coating B.

What we claim as new and desire to secure by a patent of the United States is:

1. The method of producing a photographic line print of the class described, consisting in selecting a base material capable of receiving and holding delineating marks produced by drawing or writing thereon, 35 coating said base with a basic coating of material selected from a group, said group consisting of collodion, lacquer and compounds of collodion and lacquer, placing delineating work on said basic coating by photographic 40 exposure of a light sensitive coating consisting of material including a bichromate, the portions of said basic coating between the parts of the work being made substantially bare and exposed to atmosphere, applying to the delineated work and basic coating a solvent of said basic coating material, and removing more or less of the resulting solution from the base between the parts of the work, to leave such portions of said base free for drawing or writing thereon.

2. The method of producing a photographic line print of the class described, consisting in selecting a base material capable of receiving and holding delineating marks produced by drawing or writing thereon, coating said base with a basic coating of material selected from a group, said group consisting of collodion, lacquer and compounds of collodion and lacquer, placing delineating work on said basic coating by photographic exposure of

a light sensitive coating consisting of material including a bichromate, the portions of said basic coating between the parts of the work being made substantially bare and exposed to atmosphere, applying to the delineated work and basic coating a solution of alcohol and ether to dissolve said basic coating material, and removing more or less of the resulting solution from the base between the parts of the work, to leave such portions of said base free for drawing or writing thereon.

3. An article of manufacture of the class described comprising a base consisting of a material capable of receiving and holding delineating marks produced by drawing or writing thereon, photographic line work on said base, the base being free between the lines of said line work to receive said marks, and the structure of said photographic line work comprising basic, intermediate and upper portions adhering to each other and the basic portion adhering to said base, said basic and upper portions including material chosen from a group, said group consisting of collodion, lacquer and compounds of collodion and lacquer, and said intermediate portion consisting of a fixed actinically modified substance.

4. An article of manufacture of the class described comprising a flexible base of fibrous material having a coating of starchy substance thereon capable of receiving and holding delineating marks produced by drawing or writing thereon, photographic line work on said base, the base being free between the lines of said line work to receive said marks, and the structure of said photographic line work comprising basic, intermediate and upper portions adhering together and the basic portion adhering to said base, said basic and upper portions including material chosen from a group, said group consisting of collodion, lacquer and compounds of collodion and lacquer, and said intermediate portion consisting of a fixed actinically modified substance, said basic and upper portions being mingled with said coating of starchy substance.

5. The method of producing a photographic line print of the class described, consisting in selecting a base capable of receiving and holding delineating marks produced by drawing or writing thereon, coating said base with a basic coating of material selected from a group, said group consisting of collodion, lacquer and compounds of collodion and lacquer, placing delineating work on said basic coating by photographic exposure of a light sensitive coating which coating includes a photographic bichromate and a photographic silver salt and is, where unexposed to light, soluble in water, washing the exposed surface with water to remove the chemically unmodified portion of said sensitive

solution and to leave the underlying basic coating bare, using a chemical photographic developer to bring out the delineations occasioned by the actinic action upon the sensitive coating, applying a solvent of said basic 5 coating to said developed delineations and the bare portions of said basic coating to fix said delineations and dissolve said coating, and finally removing more or less of said dissolved 10 coating, to leave the portions of said base beneath the same free for drawing or writing thereon.

6. The method of producing a photographic line print of the class described consisting 15 in selecting a base capable of receiving and holding delineating marks produced by drawing or writing thereon, coating said base with a basic coating of material selected from a group, said group consisting of collodion, lacquer and compounds of collodion and lacquer, placing delineating work on said basic coating by photographic exposure of a light 20 sensitive coating which coating includes a photographic bichromate and a photographic silver salt and is, where unexposed to light, 25 soluble in water, washing the exposed surface with water to remove the chemically unmodified portion of said sensitive solution and to leave the underlying basic coating 30 bare, using a chemical photographic developer to bring out the delineations occasioned by the actinic action upon the sensitive coating, applying to the developed delineations and the bare portions of said basic coating a solution 35 of alcohol and ether to fix said delineations and dissolve said basic coating, and finally removing more or less of said dissolved coating, to leave the portions of said base beneath the same free for drawing or writing 40 thereon.

40 In witness whereof, we hereunto subscribe our names this 1st day of July, A. D. 1929.

ARTHUR R. BAKER.  
WALTER N. BAKER.

45

50

55

60

65